

June 11, 1946.

P. FFIELD

2,402,031

METHOD OF WELDING

Filed April 3, 1940



## UNITED STATES PATENT OFFICE

2,402,031

## METHOD OF WELDING

Paul Ffield, Hingham, Mass., assignor to Bethlehem Steel Company, a corporation of Pennsylvania

Application April 3, 1940, Serial No. 327,602

4 Claims. (Cl. 113—112)

1

This invention relates to an improved steel for turbine blading which is assembled by brazing the blades to the packing pieces and also for such uses as sleeves for oil pumps and high pressure valves in which a hard wearing surface is obtained by fusing Stellite overlays onto the steel; in other words, where the metal parts are united by a process involving fusion, as by brazing, or welding. With the ordinary low carbon 12 percent chromium stainless steel which is generally used for these purposes cracking of the brazed joints and of the Stellite overlays is frequently encountered.

We have discovered that this cracking is more apt to occur when the stainless steel goes through an expansion at a relatively low temperature on cooling after brazing or welding or after welding-on the Stellite overlay. We observed that the frequency of cracking with steel in which an expansion takes place at a relatively high temperature on cooling, is much less than with steel in which an expansion takes place at a relatively low temperature. The explanation appears to be that both the brazing alloy and the Stellite are more brittle at relatively lower temperatures than at more elevated temperatures. The magnitude of the expansion also tends to be considerably greater when it occurs at the lower temperature. Thus expansion of the steel (while the packing pieces to which the turbine blades are brazed are contracting or when the Stellite overlay is contracting) at a lower temperature frequently causes cracking of the brazed joint or Stellite overlay, but expansion at a more elevated temperature does not.

Figure 1 shows dilatometer heating and cooling curves of three different steels. It will be observed that all three steels go through an expansion during cooling, but in steel A the expansion takes place at about 600° F., in steel B partly at about 1400° F. and partly at about 700° F., and in steel C the expansion occurs at about

2

1300° F. A faster rate of cooling tends to lower the temperature at which the expansion occurs. The rate of cooling in the dilatometer tests was purposely made rather fast to simulate the rate at which cooling takes place in a brazed joint of turbine blading or in a welded overlay. In this way one is safe in using the dilatometer test to ascertain whether the steel expands at an elevated temperature during cooling.

10 The compositions of the steels in Figure 1 are given below:

|         | C       | Mn      | Si      | Ni      | Cr      | Mo      | Al      |
|---------|---------|---------|---------|---------|---------|---------|---------|
|         | Percent | Percent | Percent | Percent | Percent | Percent | Percent |
| Steel A | 0.10    | 0.43    | 0.25    | 0.54    | 12.48   | 0.44    | None    |
| Steel B | .10     | .42     | .18     | .15     | 12.28   | None    | None    |
| Steel C | .09     | .20     | .27     | .13     | 12.44   | None    | .02     |

15 20 After an extended series of tests we found that when certain of the elements which may ordinarily occur in such steels as commercially produced are present in more than minimal amounts, the temperature at which the expansion on cooling occurs is lowered. Thus the presence of more than .35 percent manganese, more than .15 percent nickel, more than .15 percent copper, more than .1 percent molybdenum, and more than .1 percent carbon tended to lower the expansion temperature. On the other hand, increasing the silicon content to about .4 percent tended to counteract this. The addition of about .02 percent aluminum was particularly beneficial in raising the expansion temperature. Since sulphur combines with manganese to form manganese sulphide, the effect of increasing the sulphur content was to reduce the effect of manganese in lowering the expansion temperature.

25 30 35 As a result of these tests the following composition was found to be very suitable for turbine blading assembled by brazing or for sleeves for oil pumps and high pressure valves and other parts on which Stellite overlays are welded:

| C         | Mn        | Si        | Ni        | Cr          | Mo      | Cu        | Al          |
|-----------|-----------|-----------|-----------|-------------|---------|-----------|-------------|
| Percent   | Percent   | Percent   | Percent   | Percent     | Percent | Percent   | Percent     |
| 0.06-0.10 | 0.15-0.35 | 0.40-0.50 | 0.15 max. | 12.00-12.60 | None    | 0.15 max. | 0.025-0.035 |

1350° F. Cracks in brazed joints and in Stellite overlays are much more liable to occur in steel of types A and B than in steel of type C. The rate of cooling in these dilatometer tests was about 7° F. per minute in the neighborhood of

55 Although compositions such as those above will in general give an expansion at a high temperature on cooling, still it is desirable to ascertain this. Only such steels should be used for the purposes described above which have been tested by

the dilatometer test and actually found to give an expansion at above 1300° F.

Having thus described my invention what I claim as new and desire to secure by Letters Patent is:

1. In a method of making an article comprising at least two pieces of metal, at least one of such pieces being of steel containing 11 to 15% chromium, and the balance mainly of iron, ascertaining the expansion which takes place on cooling from a brazing or welding temperature of the steel containing 11 to 15% chromium, and uniting the metal pieces by welding or brazing, utilizing the chromium-bearing steel which has been ascertained to have an expansion above about 1300° F.

2. In a method of making turbine blading assembled by brazing or welding, and containing up to about 0.1% carbon, about 11 to 15% chromium, and the balance mainly of iron, the steps of ascertaining the expansion of the steel which takes place on cooling as after brazing or weld-

ing, and brazing or welding to produce the turbine blading utilizing the steel whose expansion takes place on cooling above about 1300° F.

3. In a method of making articles on which overlays are welded, said article containing up to about 0.1% carbon, about 11 to 15% chromium, and the balance mainly of iron, the steps of ascertaining the expansion which takes place on cooling as after the welding operation, and welding the overlays on the chromium steel whose expansion on cooling after the welding-on operation is above 1300° F.

4. In a method of making articles on which Stellite overlays are welded, said article containing up to about 0.1% carbon, about 11 to 15% chromium, and the balance mainly of iron, the steps of ascertaining the expansion which takes place on cooling as after the welding operation, and welding the overlays on the chromium steel whose expansion on cooling after the welding-on operation is above 1300° F.

PAUL FFIELD.